

## UNITED STATES PATENT OFFICE

HARRY L. BRADEN, OF YOUNGSTOWN, OHIO

## MOLD WASH

No Drawing.

Application filed August 3, 1927. Serial No. 210,465.

In casting molten metal it has long been the practice to coat the mold prior to casting with various compounds for the purpose of protecting the mold, improving the surface of the casting and facilitating the separation of the casting from the mold after the casting has become sufficiently solid to permit its removal therefrom. These compounds are ordinarily referred to as mold washes and the present invention relates thereto.

5

10

15

20

25

30

Little is known about the exact reaction occurring at the point of contact of the molten metal, and the coating of mold wash during the casting operation. It is thought by some that the carbonaceous washes burning away ahead of the metal produce a reducing atmosphere thereby reducing the oxidation on the surface of the metal and thus tending to make it more fluid, while others think that the wash partly distills or burns away as just described but that it leaves a coating of graphite or coke which enters the metal, producing a slight increase in carbon, which, however, is probably only temporary, at the surface of the metal and thereby renders it more fluid. In any case it is believed that the fluidity of the metal around the mold and adjacent its point of contact therewith is an important factor in producing a smooth, sound casting.

It is common steel mill practice to teem molten steel into metal molds in the production of steel ingots, the molds being filled with molten metal while their temperature is at any point between atmospheric or room temperature and 400° centigrade or even higher. When a mold wash is employed, the molds are coated therewith prior to the teeming operation and while within a similar temperature range, the length of time between the application of the wash and the teeming of the metal being anything from a few minutes to two hours or more. Upon the application of the wash to the mold a certain amount of the more volatile constituents of the wash are distilled off in accordance with the temperature of the mold thereby leaving the heavier, relatively less volatile constituents to form the residual coating on the mold,

and I have found that the amount of the residual coating has a material effect on the behavior of the steel or other metal when teemed into the mold, castings having defective surfaces being produced if either too much or too little of this residual coating is present. The defects in the surfaces of the castings due to these conditions cannot well be removed in subsequent operations upon the ingot.

60

65

70

75

80

85

90

95

100

I have found it possible, in accordance with the present invention, to compound a mold wash of such ingredients and in such manner that when applied to a mold when the latter is at a predetermined temperature, the quantity or amount of residual coating which is ultimately left or deposited on the mold may be controlled within practical limits, in consequence of which it is possible to form on the surface of the mold a residual coating having suitable characteristics to produce a high quality of casting having smooth, sound surfaces.

As the principal ingredient or base for my improved mold wash, I utilize a suitable hydrocarbon having a high decomposition temperature and for this purpose prefer to employ crude tar either alone or mixed with dehydrated tar, partially distilled tar, pitch or other resinous materials. Natural or artificial asphalts or petroleum still residues as well as fatty oils and waxes of vegetable origin may also be employed as bases for the wash. However, I have found that good results may be obtained from the use of crude tar, and as this material is relatively cheap and readily procurable I prefer to utilize it under most conditions.

This hydrocarbon base is mixed in any convenient manner with a suitable solvent or thinner and for this purpose I prefer to employ creosote oil although if desired other like oils or tar oil fractions, rosin oil, paint thinners or petroleum oils of proper volatility and solvent action may be employed. However, as in the case of the crude tar, creosote oil is a readily obtainable and relatively cheap material and I therefore prefer to employ it as the solvent under most conditions.

When the mold wash is to be heated before being applied to the mold the addition of any other ingredients beside the base and the solvent is unnecessary, the heating rendering the wash sufficiently fluid for convenient application but when the wash is to be applied cold, that is, substantially at room temperature, I prefer, with a view to rendering the wash sufficiently fluid for convenient application, to add a suitable quantity of naphthalene which material as is well known, progressively increases the fluidity of tar when added thereto in a quantity up to about 20% of the total weight of the mixture, maximum fluidity being attained at this point.

As the several ingredients of the wash all contain more or less volatile ingredients or fractions which distill off in the presence of heat, I therefore, in preparing my mold wash, so calculate the proportions of the ingredients as to bring about the deposit of a predetermined residual coating on the mold surface when the wash is applied to the mold when the latter is at a given temperature. Thus, if the wash is to be applied to the molds at atmospheric or room temperature, under which conditions there will be a relatively small loss of the volatile constituents by distillation from the heat of the mold, I so determine the proportions of the ingredients in the wash that the ultimate coating on the mold will conform to the desired condition while, on the other hand, if the wash is to be applied to the mold when the latter is very hot as, for example, 400° centigrade or even higher, I may so proportion the ingredients of the wash that the ultimate residual coating after the relatively great distillation and volatilization of ingredients of the wash effected by the heat of the mold has taken place will conform to substantially like conditions.

Thus, with this end in view, in compounding the wash I take any convenient mold temperature as a guide, for example, 400° centigrade, and then distill at this temperature, preferably separately, samples of the several ingredients of which the wash is to be composed and which embody fractions volatilizable at or below that temperature and note the residual percentages of the ingredients after such distillation is effected. From the data thus obtained the relative quantities of the different ingredients to be included in the mold wash may be readily calculated so as to produce a wash from which, when it is applied to the mold at a temperature substantially corresponding to that at which the distillation of the samples was effected, a definite percentage or fraction of the whole quantity employed will be volatilized by the heat of the mold, thus leaving the desired amount of residual coating thereon.

As an example of one manner of compounding my mold wash from tar and creosote oil in accordance with the present invention, it may be assumed that the wash is to be applied to the molds when the latter are at a temperature of approximately 400° centigrade and that it is desired to leave on the mold a residual coating of substantially 37% of the total amount of wash employed, this percentage having been found in practice to give very satisfactory results. Under these conditions samples of both the tar and the creosote oil may be distilled separately at 400° centigrade and the percentages of residuum of each sample at the termination of the distilling operation duly noted. From these percentages the quantity of each ingredient which must be used to produce the desired residual percentage of 37% may be readily calculated and the mold wash then compounded from the ingredients in corresponding proportions which, in the present example, will approximate 75% by volume of tar and 25% by volume of creosote oil.

It will of course be understood that if a greater or lesser amount of residual coating is desired on the mold when the latter is to be coated at the assumed temperature of 400° centigrade, the proportions of the ingredients will be correspondingly varied and, equally, that if the molds are to be coated at some other temperature, either higher or lower, than 400° centigrade the distillation of the samples of the ingredients will be effected at such temperature and the proper proportions of the ingredients which are to be compounded to form the wash determined from the percentage of residua of the several ingredients as ascertained by such test distillation.

When the mold wash is intended to be applied to the molds without preheating the wash, the addition of naphthalene is desirable to render the wash sufficiently fluid for convenient application; fluidity being particularly advantageous when the wash is to be applied to the molds by spraying. Under these conditions consideration must also be given to the effect of the naphthalene which is added as well as to the naphthalene fractions of the tar or other base and of the creosote oil or other thinner or solvent in determining the proper proportions of the ingredients of the ultimate mixture when calculating the same from the residua left after distillation of the test samples.

Powdered graphite may sometimes be added to the wash with beneficial results in quantities running up to approximately 20% of the total volume of the latter while, if desired, addition may also be made of fire extinguishing chemicals such as carbontetrachloride for the purpose of reducing the fire hazard.

The wash prepared as hereinbefore described may be applied to the molds in any convenient way as by means of a brush or by

70  
75  
80  
85  
90  
95  
100  
105  
110  
115  
120  
125  
130  
135

sote oil in accordance with the present invention, it may be assumed that the wash is to be applied to the molds when the latter are at a temperature of approximately 400° centigrade and that it is desired to leave on the mold a residual coating of substantially 37% of the total amount of wash employed, this percentage having been found in practice to give very satisfactory results. Under these conditions samples of both the tar and the creosote oil may be distilled separately at 400° centigrade and the percentages of residuum of each sample at the termination of the distilling operation duly noted. From these percentages the quantity of each ingredient which must be used to produce the desired residual percentage of 37% may be readily calculated and the mold wash then compounded from the ingredients in corresponding proportions which, in the present example, will approximate 75% by volume of tar and 25% by volume of creosote oil.

It will of course be understood that if a greater or lesser amount of residual coating is desired on the mold when the latter is to be coated at the assumed temperature of 400° centigrade, the proportions of the ingredients will be correspondingly varied and, equally, that if the molds are to be coated at some other temperature, either higher or lower, than 400° centigrade the distillation of the samples of the ingredients will be effected at such temperature and the proper proportions of the ingredients which are to be compounded to form the wash determined from the percentage of residua of the several ingredients as ascertained by such test distillation.

When the mold wash is intended to be applied to the molds without preheating the wash, the addition of naphthalene is desirable to render the wash sufficiently fluid for convenient application; fluidity being particularly advantageous when the wash is to be applied to the molds by spraying. Under these conditions consideration must also be given to the effect of the naphthalene which is added as well as to the naphthalene fractions of the tar or other base and of the creosote oil or other thinner or solvent in determining the proper proportions of the ingredients of the ultimate mixture when calculating the same from the residua left after distillation of the test samples.

Powdered graphite may sometimes be added to the wash with beneficial results in quantities running up to approximately 20% of the total volume of the latter while, if desired, addition may also be made of fire extinguishing chemicals such as carbontetrachloride for the purpose of reducing the fire hazard.

The wash prepared as hereinbefore described may be applied to the molds in any convenient way as by means of a brush or by

a suitable spraying apparatus and either considerably in advance of the time when the metal is to be teemed into the molds or only a short time in advance thereof, the coating 5 being preferably made as uniform as possible and of substantially even thickness in accordance with the usual practice.

While my improved mold wash is especially suited for use upon metallic molds in which 10 steel is to be cast, it may be used with beneficial results on other forms of molds designed for the reception of molten steel or on metallic or other molds in the casting of metals other than steel such, for example, 15 as cast iron. Furthermore, while I have referred more particularly to certain ingredients which I prefer to use in compounding the wash, it will be understood that I do not specifically limit myself to the use thereof 20 as other ingredients having substantially similar characteristics may be employed if desired.

Having thus described my invention in such manner as to enable those skilled in the 25 art to readily comprehend and practise the same, I claim and desire to protect by Letters Patent of the United States:

1. A mold wash intended for application to the surfaces of molds in which metal is to 30 be cast, comprising a hydrocarbon base having a high decomposition temperature and creosote oil.
2. A mold wash intended for application to the surfaces of molds in which metal is to 35 be cast, comprising tar and creosote oil.
3. A mold wash intended for application to the surfaces of molds in which metal is to be cast, comprising a hydrocarbon base having a high decomposition temperature, creo- 40 sote oil and naphthalene.
4. A mold wash intended for application to the surfaces of molds in which metal is to be cast, comprising tar, creosote oil and naphthalene.
- 45 5. A mold wash intended for application to the surfaces of molds in which metal is to be cast, comprising substantially 75% by volume of tar and 25% by volume of creosote oil.

50 In witness whereof, I have hereunto set my hand this 22nd day of July, 1927.

HARRY L. BRADEN.